

# United States Patent [19]

Gregory et al.

[11] Patent Number: 4,968,657

[45] Date of Patent: Nov. 6, 1990

## [54] THERMAL TRANSFER PRINTING

[75] Inventors: Peter Gregory, Bolton; Roy Bradbury, Widnes, both of England

[73] Assignee: Imperial Chemical Industries plc, London, England

[21] Appl. No.: 342,018

[22] Filed: Apr. 24, 1989

## Related U.S. Application Data

[63] Continuation of Ser. No. 227,913, Aug. 3, 1988, abandoned.

## [30] Foreign Application Priority Data

Aug. 4, 1987 [GB] United Kingdom ..... 8718429  
May 13, 1988 [GB] United Kingdom ..... 8811437.6

[51] Int. Cl.<sup>5</sup> ..... B41M 5/035; B41M 5/26

[52] U.S. Cl. ..... 503/227; 8/471;  
428/195; 428/913; 428/914

[58] Field of Search ..... 8/471; 428/913, 914,  
428/195; 503/227

## [56] References Cited

### FOREIGN PATENT DOCUMENTS

0247737 12/1987 European Pat. Off.  
60-27594 2/1985 Japan ..... 503/227  
61-244595 10/1986 Japan ..... 503/227  
2159971 12/1985 United Kingdom .

### OTHER PUBLICATIONS

European Search Report, Application No. EP 88 30 6645.

Abstract, JP-A-60 27 594, vol. 9, No. 152 (1985).

Abstract, JP-A-61 268 494, vol. 11, No. 115 (1986).

Chemical Abstract, J6 27594A, "Heat-Sensitive Transfer Recording Material—Based on Pyrido Azo Series Dye." Mitsubishi.

Chemical Abstract, J6 1244595A, "Dye for Heat-Sensitive Transfer Recording—Comprises Cyano-Hydroxy-Pyridone-Azo-Phenyl Deriv." Mitsubishi.

Chemical Abstract, J6 152563A, "Pyridone Azo Series Heat-Sensitive Recording Dye—Stable to Light, Moisture and Chemicals." Mitsubishi.

Chemical Abstract, J6 1 262191A, "Sublimation Trans-

fer Material—Contains 5-phenyl:azo-4-methyl 6-hydroxy Pyridin 2-one Deriv. as Dye.", Sumitomo.

Chemical Abstract, J63 39380A, "Heat-Sensitive Transfer Sheet—Contains Pyridone-Azo Series Dye on Base Film, for Sublimation Type Heat-Sensitive Recording", Mitsubishi.

Chemical Abstracts, J61 12393A, "Yellow Series Heat-Transfer Coloring Material—Comprises Pyridyl Mono-Azo Benzoate Deriv.", Mitsui Toatsu.

Chemical Abstract, J61 12394A, "Yellow Heat-Transfer Coloring Material—Comprises Pyrazole Diazo Cpd. Used in Transfer Printing Synthetic Fibre and Transfer Heat Recording." Mitsui Toatsu.

Primary Examiner—Bruce H. Hess

Attorney, Agent, or Firm—Cushman, Darby & Cushman

## [57] ABSTRACT

A thermal transfer printing sheet, suitable for use in a thermal transfer printing process, comprising a substrate having a coating comprising a dye of the formula:



wherein

X represents nitro or —COOR<sup>1</sup> in which R<sup>1</sup> is an optionally substituted hydrocarbyl radical;

Y represents an optionally substituted C<sub>1-10</sub>-alkyl or alkoxy radical;

Z represents an alkyl radical, and

R represents an alkyl radical which may be interrupted by one or two —O— or —COO— links.

6 Claims, No Drawings

## THERMAL TRANSFER PRINTING

This is a continuation of application Ser. No. 07/227,913, filed Aug. 3, 1988, now abandoned.

## INTRODUCTION

This specification describes an invention relating to thermal transfer printing (TTP), especially to a TTP sheet carrying a dye or dye mixture, and to a transfer printing process in which dye is transferred from the transfer sheet to a receiver sheet by the application of heat.

In TTP a heat-transferable dye is applied to a sheet-like substrate in the form of an ink, usually containing a 15 polymeric or resinous binder to bind the dye to the substrate, to form a transfer sheet. This is then placed in contact with the material to be printed, (generally a film of polymeric material such as a polyester sheet) herein-after called the receiver sheet and selectively heated in accordance with a pattern information signal whereby dye from the selectively heated regions of the transfer sheet is transferred to the receiver sheet and forms a pattern thereon in accordance with the pattern of heat applied to the transfer sheet.

Important criteria in the selection of a dye for TTP are its thermal properties, brightness of shade, fastness properties, such as light fastness, and facility for application to the substrate in the preparation of the transfer sheet. For suitable performance the dye should transfer evenly, in proportion to the heat applied to the TTP sheet so that the depth of shade on the receiver sheet is proportional to the heat applied and a true grey scale of coloration can be achieved on the receiver sheet. Brightness of shade is important in order to achieve as wide a range of shades with the three primary dye shades of yellow, magenta and cyan. As the dye must be sufficiently mobile to migrate from the transfer sheet to the receiver sheet at the temperatures employed, 300°-400° C., it is generally free from ionic and water-solubilising groups, and is thus not readily soluble in aqueous or water-miscible media, such as water and ethanol. Many suitable dyes are also not readily soluble in the hydrocarbon solvents which are commonly used in, and thus acceptable to, the printing industry; for 45 example, alcohols such as i-propanol, ketones such as methyl-ethylketone (MEK), methyl-i-butylketone (MIBK) and cyclohexanone, aromatic hydrocarbons such as toluene and ethers such as tetrahydrofuran. Although the dye can be applied as a dispersion in a 50 suitable solvent, it has been found that brighter, glossier and smoother final prints can be achieved on the receiver sheet if the dye is applied to the substrate from a solution. In order to achieve the potential for a deep shade on the receiver sheet it is desirable that the dye 55 should be readily soluble in the ink medium. It is also important that a dye which has been applied to a transfer sheet from a solution should be resistant to crystallisation so that it remains as an amorphous layer on the transfer sheet for a considerable time.

The following combination of properties are highly desirable for a dye which is to be used in TTP:

Ideal spectral characteristics (narrow absorption curve with absorption maximum matching a photographic filter: for yellow dyes, a blue filter).

High tinctorial strength.

Correct thermochemical properties (high thermal stability and good transferability with heat).

High optical densities on printing.

Good solubility in solvents acceptable to printing industry: this is desirable to produce solution coated dyesheets.

5 Stable dyesheets (resistant to dye migration or crystallisation).

Stable printed images on the receiver sheet (to heat and especially light).

The achievement of good light fastness in TTP is 10 extremely difficult because of the unfavourable environment of the dye, namely surface printed polyéster on a white pigmented base. Many known dyes for polyester fibre with high light fastness (>6 on the International Scale of 1-8) on polyester fibre exhibit very poor light fastness (<3) in TTP.

The achievement of the desirable properties with 15 yellow dyes is particularly difficult and the leading yellow dyes for the conventional transfer printing of polyester textile materials do not meet these criteria.

20 For example, CI Disperse Yellow 3, an azophenol dye, does not have the correct spectral characteristics (too red and dull), has poor solubility (precludes solution coated dyesheets), is tinctorially weak (gives low optical density on printing) and has poor light fastness. CI

25 Disperse Yellow 54, a quinophthalone dye which is probably the leading yellow dye for the conventional transfer printing of polyester textile materials, has very poor solubility which precludes its use for solution coated dyesheets.

It has now been found that certain azopyridone dyes 30 have properties which render them more suitable for TTP than dyes which have previously been known or proposed for the heat transfer printing of textile materials. In particular, the dyes provide reddish-yellow shades of high light fastness very suitable for skin tones. In addition to their high tinctorial strength, the dyes are characterised by good solubility providing very stable dyesheets.

## THE INVENTION

According to a first aspect of the present invention there is provided a thermal transfer printing sheet comprising a substrate having a coating comprising a dye of the formula:



wherein

X represents nitro or  $-\text{COOR}^1$  in which  $\text{R}^1$  is an optionally substituted hydrocarbyl radical;

Y represents an optionally substituted  $\text{C}_{1-10}$ -alkyl or 60 alkoxy radical;

Z represents an alkyl radical, and

R represents an alkyl radical which may be interrupted by one or two  $-\text{O}-$  or  $-\text{COO}-$  links.

## THE COATING

The coating preferably comprises a binder and one or more dyes of Formula I. The ratio of binder to dye is preferably at least 1:1 and more preferably from 1.5:1 to

4:1 in order to provide good adhesion between the dye and the substrate and inhibit migration of the dye during storage.

The coating may also contain other additives, such as curing agents, preservatives, etc., these and other ingredients being described more fully in EP Nos. 133011A, 133012A and 111004A.

### THE BINDER

The binder may be any resinous or polymeric material suitable for binding the dye to the substrate which has acceptable solubility in the ink medium, i.e. the medium in which the dye and binder are applied to the transfer sheet. Examples of binders include cellulose derivatives, such as ethylhydroxyethylcellulose (EHEC), hydroxypropylcellulose (HPC), ethylcellulose, methylcellulose, cellulose acetate and cellulose acetate butyrate; carbohydrate derivatives, such as starch; alginic acid derivatives; alkyd resins; vinyl resins and derivatives, such as polyvinyl alcohol, polyvinyl acetate, polyvinyl butyral and polyvinyl pyrrolidone; polymers and co-polymers derived from acrylates and acrylate derivatives, such as polyacrylic acid, polymethyl methacrylate and styrene-acrylate copolymers, polyester resins, polyamide resins, such as melamines; polyurea and polyurethane resins; organosilicones, such as polysiloxanes, epoxy resins and natural resins, such as gum tragacanth and gum arabic.

It is however preferred to use a binder which is soluble in one of the above-mentioned commercially acceptable organic solvents. Preferred binders of this type are EHEC, particularly the low and extra-low viscosity grades, and ethyl cellulose.

### THE DYE OF FORMULA I

Formula I is written in the hydrazone tautomeric form because the dye is believed to exist in this form (see Lycka and Machacek, in *Dyes and Pigments 1986*, 171).

It is preferred that X is a nitro group. Examples of 40 optionally substituted hydrocarbyl radicals which may be represented by R<sup>1</sup> when X is a —COOR<sup>1</sup> group include alkyl radicals, for example C<sub>1-4</sub>-alkyl radicals, and aralkyl radicals, for example, phenyl-C<sub>1-4</sub>-alkyl radicals.

Examples of substituents which may be present in the optionally substituted alkyl or alkoxy radicals represented by Y include electron withdrawing groups such as cyano or alkoxy carbonyl which are preferably separated from the aromatic ring by at least two carbon atoms. It is preferred that Y is a C<sub>1-6</sub>, for example a C<sub>3-5</sub>, alkyl or alkoxy radical although methyl might be preferred on cost grounds.

Z is preferably an unbranched C<sub>1-4</sub>-alkyl radical, especially methyl.

It is preferred that R is a C<sub>1-11</sub>-alkyl radical, unbranched at the 2-position relative to the ring nitrogen, especially a C<sub>2-4</sub> and more especially a C<sub>3</sub> alkyl radical.

The dye of Formula I has particularly good thermal properties giving rise to even prints on the receiver sheet, the depth of shade being accurately proportional to the quantity of applied heat so that a true grey scale of coloration can be attained.

The dye of Formula I also has strong coloristic properties and good solubility in a wide range of solvents, especially those solvents which are widely used and accepted in the printing industry, for example, alkanols, such as i-propanol & butanol; aromatic hydrocarbons,

such as toluene, ketones such as MEK, MIBK and cyclohexanone and ethers such as tetrahydrofuran. This produces inks (solvent plus dye and binder) which are stable and allow production of solution coated dye-sheets. The latter are stable, being resistant to dye crystallisation or migration during prolonged storage.

The combination of strong coloristic properties and good solubility in the preferred solvents allows the achievement of deep, even shades on the receiver sheet.

10 The receiver sheets according to the present invention have bright, strong and even yellow shades which are fast to both light and heat.

### THE SUBSTRATE

The substrate may be any convenient sheet material capable of withstanding the temperatures involved in TTP, up to 400° C. over a period of up to 20 milliseconds (msec) yet thin enough to transmit heat applied on one side through to the dye on the other side to effect transfer to a receiver sheet within such short periods, typically from 1-10 msec. Examples of suitable materials are paper, especially high quality paper of even thickness, such as capacitor paper, polyester, polyacrylate, polyamide, cellulosic and polyalkylene films, metallised forms thereof, including co-polymer and laminated films, especially laminates incorporating a polyester receptor layer on which the dye is deposited. Such laminates preferably comprise, a backcoat, on the opposite side of the laminate from the receptor layer, of a heat resistant material, such as a thermosetting resin, e.g. a silicone, acrylate or polyurethane resin, to separate the heat source from the polyester and prevent melting of the latter during the thermal transfer printing operation. The thickness of the substrate may vary within wide limits depending upon its thermal characteristics but is preferably less than 50 µm and more preferably below 10 µm.

### THE TTP PROCESS

According to a further feature of the present invention there is provided a transfer printing process which comprises contacting a transfer sheet coated with a dye of Formula I with a receiver sheet, so that the dye is in contact with the receiver sheet and selectively heating 45 areas of the transfer sheet whereby dye in the heated areas of the transfer sheet may be selectively transferred to the receiver sheet.

The transfer sheet is preferably heated to a temperature from 250° C. to 400° C., more preferably above 300° C. and especially around 350° C., for a period of from 1 to 10 milliseconds while it is maintained with the coating in contact with the receiver sheet. The depth of shade of print on any area of the receiver sheet will vary with the time period for which the transfer sheet is heated while in contact with that area of the receiver sheet.

### THE RECEIVER SHEET

The receiver sheet conveniently comprises a polyester sheet material, especially a white polyester film, preferably of polyethylene terephthalate (PET). Although some dyes of Formula I are known for the coloration of textile materials made from PET, the coloration of textile materials, by dyeing or printing is carried out under such conditions of time and temperature that the dye can penetrate into the PET and become fixed therein. In thermal transfer printing, the time period is so short that penetration of the PET is much less effec-

tive and the substrate is preferably provided with a receptive layer, on the side to which the dye is applied, into which the dye more readily diffuses to form a stable image. Such a receptive layer, which may be applied by co-extrusion or solution coating techniques, may comprise a thin layer of a modified polyester or a different polymeric material which is more permeable to the dye than the PET substrate. While the nature of the receptive layer will affect to some extent the depth of shade and quality of the print obtained it has been found that the dyes of Formula I give particularly strong and good quality prints (e.g. fast to light, heat and storage) on any specific transfer or receiver sheet, compared with other dyes of similar structure which have been proposed for thermal transfer printing. The design of receiver and transfer sheets is discussed further in EP Nos. 133,011 and 133,012.

The invention is further illustrated by the following examples in which all parts and percentages are by weight unless otherwise indicated.

### EXAMPLE 1

Ink 1 was prepared by dissolving 0.1 g of Dye 1 in 5 ml chloroform and adding 9.5 ml of a 2.7% solution of EHEC-elv in chloroform. The ink was stirred until 25 homogeneous.

A second ink (Ink 2) was prepared by the same method using Dye 2.

Dyes 1 and 2 are identified in the following Table by the substituents present in Formula I.

|       | X               | Y               | Z               | R               | max | ECmax |
|-------|-----------------|-----------------|-----------------|-----------------|-----|-------|
| Dye 1 | NO <sub>2</sub> | CH <sub>3</sub> | CH <sub>3</sub> | CH <sub>3</sub> | 449 | 38200 |

| X                                             |
|-----------------------------------------------|
| NO <sub>2</sub>                               |
| NO <sub>2</sub>                               |
| NO <sub>2</sub>                               |
| NO <sub>2</sub>                               |
| NO <sub>2</sub>                               |
| NO <sub>2</sub>                               |
| NO <sub>2</sub>                               |
| NO <sub>2</sub>                               |
| NO <sub>2</sub>                               |
| NO <sub>2</sub>                               |
| NO <sub>2</sub>                               |
| CO <sub>2</sub> C <sub>2</sub> H <sub>5</sub> |
| NO <sub>2</sub>                               |
| NO <sub>2</sub>                               |
| NO <sub>2</sub>                               |

A transfer sheet was prepared by applying Ink 1 to a sheet of  $6\mu$  thick polyethylene terephthalate using a wire-wound metal Meyer-bar to produce a 24 micron wet film of ink on the surface of the sheet. The ink was dried with hot air and the sheet is hereinafter referred to as **TS 1**.

A second transfer sheet was prepared in the same way using Ink 2 in place of Ink 1. This transfer sheet is 60 hereinafter referred to as TS 2.

A sample of TS 1 was sandwiched with a receiver sheet, comprising a composite structure based on a white polyester base having a receptive coating layer on the side in contact with the printed surface of TS 1. The 65 sandwich was placed on the drum of a transfer printing machine and passed over a matrix of closely-spaced pixels which were selectively heated in accordance

with a pattern information signal to a temperature of  $>300^{\circ}$  C. for periods from 2 to 10 msec, whereby a quantity of the dye, in proportion to the heating period, at the position on the transfer sheet in contact with a pixel while it was hot was transferred from the transfer sheet to the receiver sheet. After passage over the array of pixels the transfer sheet was separated from the receiver sheet. The printed receiver sheet is hereinafter referred to as RS 1.

Receiver sheet RS 2 was prepared in the same way using transfer sheet TS 2 in place of TS 1.

The stability of each ink and the quality of the print on the transfer sheet was assessed by visual inspection. An ink was considered stable if there was no precipitation over a period of two weeks at ambient and a transfer sheet was considered stable if it remained substantially free from crystallisation for a similar period. The quality of the printed impression on the receiver sheet was assessed in respect of reflected colour density by means of a densitometer (Sakura Digital densitometer). The results of the assessments are set out below.

|      | Optical Density | Light Fastness |
|------|-----------------|----------------|
| RS 1 | 1.3             | 4              |
| RS 2 | 1.2             | 5              |

**EXAMPLE 2**

30 Other dyes, identified in the following Table by the substituents present in Formula I, were used in the preparation of inks, transfer sheets and receiver sheets as described in Example 1. The results obtained are set out in the Table.

TABLE

| X                                             | Y                                | R                                              | Z                               | OD   | LF     | max (max)    |
|-----------------------------------------------|----------------------------------|------------------------------------------------|---------------------------------|------|--------|--------------|
| NO <sub>2</sub>                               | t-C <sub>4</sub> H <sub>9</sub>  | n-C <sub>3</sub> H <sub>7</sub>                | n-C <sub>3</sub> H <sub>7</sub> | 1.25 | 4      | 450 (39,153) |
| NO <sub>2</sub>                               | n-C <sub>4</sub> H <sub>9</sub>  | n-C <sub>3</sub> H <sub>7</sub>                | n-C <sub>3</sub> H <sub>7</sub> | 1.26 | 3-4(4) | 450 (43,514) |
| NO <sub>2</sub>                               | CH <sub>3</sub>                  | n-C <sub>2</sub> H <sub>7</sub>                | n-C <sub>3</sub> H <sub>7</sub> | 1.37 | 4      | 448 (38,761) |
| NO <sub>2</sub>                               | t-C <sub>4</sub> H <sub>9</sub>  | n-C <sub>3</sub> H <sub>7</sub>                | CH <sub>3</sub>                 | 1.24 | 3-4(4) | 448 (42,255) |
| NO <sub>2</sub>                               | n-C <sub>9</sub> H <sub>19</sub> | n-C <sub>5</sub> H <sub>11</sub>               | CH <sub>3</sub>                 | 0.97 | 3-4(4) | 450 (40,036) |
| NO <sub>2</sub>                               | n-C <sub>9</sub> H <sub>19</sub> | CH <sub>3</sub>                                | CH <sub>3</sub>                 | 1.13 | 3-4(4) | 450 (39,554) |
| NO <sub>2</sub>                               | CH <sub>3</sub>                  | CH <sub>3</sub>                                | CH <sub>3</sub>                 | 1.46 | 4      |              |
| NO <sub>2</sub>                               | CH <sub>3</sub>                  | n-C <sub>3</sub> H <sub>7</sub>                | CH <sub>3</sub>                 | 1.65 | 4      | 450          |
| NO <sub>2</sub>                               | n-C <sub>3</sub> H <sub>7</sub>  | n-C <sub>3</sub> H <sub>7</sub>                | CH <sub>3</sub>                 | 1.45 |        |              |
| NO <sub>2</sub>                               | n-C <sub>4</sub> H <sub>9</sub>  | CH <sub>3</sub>                                | CH <sub>3</sub>                 | 1.18 | 4      |              |
| NO <sub>2</sub>                               | CH <sub>3</sub>                  | CH <sub>2</sub> OC <sub>2</sub> H <sub>5</sub> | CH <sub>3</sub>                 | 1.33 | 4      |              |
| CO <sub>2</sub> C <sub>2</sub> H <sub>5</sub> | CH <sub>3</sub>                  | n-C <sub>3</sub> H <sub>7</sub>                | CH <sub>3</sub>                 | 1.68 | 3      | 442 (32,457) |
| NO <sub>2</sub>                               | t-C <sub>4</sub> H <sub>9</sub>  | n-C <sub>5</sub> H <sub>11</sub>               | CH <sub>3</sub>                 | 1.14 | 4      | 448 (39,916) |
| NO <sub>2</sub>                               | CH <sub>3</sub>                  | n-C <sub>11</sub> H <sub>23</sub>              | CH <sub>3</sub>                 | 1.13 | 3-4(4) | 448 (34,033) |
| NO <sub>2</sub>                               | CH <sub>3</sub>                  | n-C <sub>7</sub> H <sub>15</sub>               | CH <sub>3</sub>                 | 1.33 | 4      | 446 (38,161) |

Dye 2       $\text{NO}_2$        $\text{CH}_3$        $\text{CH}_3$        $n\text{-C}_3\text{H}_7$       450      36000

**What is claimed is:**

1. A thermal transfer printing sheet comprising a substrate having a coating comprising a binder, and a dye of the formula:



wherein

X represents nitro or  $-\text{COOR}^1$  in which  $\text{R}^1$  is an optionally substituted hydrocarbyl radical;

Y represents an optionally substituted  $\text{C}_{1-10}$ -alkyl or  $\text{C}_{1-10}$ -alkoxy radical;

Z represents an alkyl radical, and

R represents a  $\text{C}_1$ ,  $\text{C}_2$ , or  $\text{C}_3$ -alkyl radical which may be interrupted by one or two  $-\text{O}-$  or  $-\text{COO}-$  links.

2. A thermal transfer printing sheet according to claim 1, wherein, in the dye, Y is a  $\text{C}_{1-6}$ -alkyl or  $\text{C}_{1-6}$ -alkoxy radical.

3. A thermal transfer printing sheet according to claim 1, wherein, in the dye, Z is an unbranched  $\text{C}_{1-4}$ -alkyl radical.

4. A thermal transfer printing sheet according to claim 3 wherein Z is methyl.

5. A thermal transfer printing sheet according to claim 1, wherein R is  $\text{n-C}_3\text{H}_7$ .

10 6. A thermal transfer printing process which comprises contacting a transfer sheet according to claim 1, with a receiver sheet, so that the dye is in contact with the receiver sheet and selectively heating areas of the transfer sheet whereby dye in the heated areas of the transfer sheet is selectively transferred to the receiver sheet.

\* \* \* \* \*